

April 14, 1931.

C. J. WRIGHT

1,800,239

MANUFACTURE OF LEAD OXIDES

Filed Sept. 17, 1925

Fig. 2.



## UNITED STATES PATENT OFFICE

CARL J. WRIGHT, OF WEST NEW BRIGHTON, NEW YORK, ASSIGNOR TO COMBUSTION UTILITIES CORPORATION, OF NEW YORK, N. Y., A CORPORATION OF MAINE

## MANUFACTURE OF LEAD OXIDES

Application filed September 17, 1925. Serial No. 56,988.

The present invention relates to the manufacture of lead oxides and more particularly to the manufacture of red lead pigment.

According to the present invention, molten lead is agitated in contact with a current of heated air with the formation of lead monoxide. In case the final product is to be red lead, the monoxide of lead formed as just stated, is then further agitated in contact with a current of heated gas derived at least in part from the same current as that involved in forming the monoxide to convert the monoxide into red lead pigment.

It is one of the objects of the present invention to provide a method of forming lead oxides which shall be rapid and also require a small amount of labor.

A further object of the present invention is to provide an apparatus suitable for carrying out the process just mentioned.

It is known that lead monoxide forms from molten lead at a temperature of about 700° F. It is known, moreover, that in the manufacture of red lead from lead monoxide the oxides should not be heated above 840° F. or thereabouts. Moreover, a certain amount of heat is formed in the reaction forming lead monoxide from metallic lead and also in the reaction forming red lead from lead monoxide. The process and apparatus according to the present invention are designed to operate consistently with the facts as just stated.

Further objects and advantages of the process and apparatus according to the present invention will be apparent to those skilled in the art from the following description taken in connection with the accompanying drawing, in which

Fig. 1 is an elevation of an apparatus according to the present invention and adapted to carry out the process according to the present invention, parts being shown in section and parts being broken away for purposes of illustration;

Fig. 2 is a partial section taken on the line 2—2 of Fig. 1.

In the apparatus according to the present invention, and illustrated in the drawing, the metallic lead is melted by hot gases which

have first been used in forming lead oxides. Pot 10 is a receptacle in which the lead is melted as just mentioned, the body of pot 10 being held as illustrated within a chamber 12 in such position that the pot is in contact substantially over its entire surface with hot gases within the chamber 12 coming from the upper end of the rotary kiln 14. From the chamber 12, kiln gases pass to the atmosphere through a conduit 16.

The molten lead from chamber 10, however, passes downwardly through pipe 18 into the upper end of a second inclined rotary kiln 20, kiln 20 being on a lower level than kiln 14, and the pipe 18 running throughout its length through a current of hot gases contained in kilns 14 and 20 and chamber 23, the chamber 23 just mentioned serving to connect the upper end of kiln 20 with the lower end of kiln 14. Heated air at a temperature of about 800° F. is injected into the lower end of kiln 20 through a pipe or nozzle 22 and the stream of heated air thereupon passes upwardly through the inclined kilns 20 and 14 into melting chamber 12. Within kiln 20, the molten lead dropping from the lower end of pipe 18 travels downwardly through this kiln countercurrent to the upwardly flowing stream of air. Within the kiln 20, moreover, the molten lead and the lead monoxide formed therefrom are continuously agitated in contact with the air stream by being lifted and dropped repeatedly in their passage through the kiln. For the purpose of lifting and dropping the metallic lead and lead monoxide in contact with the air current as just mentioned, the interior surface of the kiln 20 is provided with a series of cells or pockets 24 covering substantially the entire inner surface of the kiln 20 and formed by two sets of intersecting ribs 26, 26 and 28, 28, projecting from the inner surface of the kiln 20, ribs 26, 26 being spaced and parallel and running longitudinally of the kiln while ribs 28, 28 are spaced and parallel and run circumferentially of the kiln 20.

The rate of travel of the metallic lead and lead monoxide downwardly through kiln 20 is determined, the inclination of the kiln having been fixed upon, by the speed of rota-

tion of the kiln. According to the present invention, the R. P. M. of kiln 20 is regulated with respect to the amount of heated air passing upwardly through the kiln so that some metallic lead is not converted into monoxide within the kiln 20, but the monoxide formed together with metallic lead falls from the lower end of kiln 20 into separating pot 30. The molten metallic lead separates from the lead monoxide and settles to the bottom of the pot 30, being drawn off therefrom through a pipe 32 whereas the lighter lead monoxide is drawn off from pot 30 at a higher level than the melted lead through a downwardly inclined chute 34. The chute 34 delivers lead monoxide to a bucket conveyer 36 by which the monoxide is elevated to a bin 38. From the bin 38 the lead monoxide is delivered preferably by gravity into the upper end of kiln 14 by pipe 40 being illustrated in Fig. 1 as connecting the bin 38 with kiln 14 for this purpose. Within kiln 14 the lead monoxide is lifted and dropped in contact with an ascending current of hot air by means of a second set of cells or pockets 24b similar to those described in connection with kiln 20. The lead monoxide is gradually converted into red lead as it passes through the kiln 14 and the red lead drops from the lower end of this kiln into a chute 42 from which it is conveyed away.

It will be obvious that lead monoxide from the pot 30 can be used as such instead of being converted into red lead. When the lead monoxide is to be so converted, however, it is important that the temperature in kiln 20 should not be permitted to rise to the point at which any of the lead monoxide is injured for the purpose of forming red lead. Certain other uses of lead monoxide also require that the temperature be regulated and kept down during the course of the manufacture of the lead monoxide. For the purpose of preventing an undesirable rise in temperature in the upper part of kiln 20, a stream of relatively cold air is introduced into the kiln 20 through pipe 44 the point of delivery of pipe 44 being preferably slightly above the mid-point of the kiln 20. The air delivered through pipe 44 not only supplies fresh oxide to the gas stream to compensate for that absorbed in the production of lead monoxide in the lower end of kiln 20, but also absorbs by its lower temperature the excess heat produced in the formation of lead monoxide from lead within kiln 20.

The gas stream from the upper end of kiln 20 passes into the lower end of kiln 14 through the chamber 23 and in order to prevent the temperature of the gases in kiln 14 from rising to the point at which red lead formation is interfered with, it is preferred to introduce into the chamber 23 an additional supply of relatively cold air through the pipe 46. Pipes 44 and 46 are

provided with valves 45 and 47 respectively as illustrated whereby the amount of cooling air delivered through these pipes may be regulated to produce the desired results in kilns 14 and 20.

Heated air from the nozzle 22 to be injected into the lower end of kiln 20 may be supplied conveniently by forcing air through a coil of pipe 48 contained in a stack 50. Stack 50 may be conveniently arranged above a chamber 31 surrounding the lower end of kiln 20 and in which the pot 30 is placed. Heating gases for producing the desired temperature of the coil 48 may be introduced into the stack 50 through a passage 52 leading from the furnace 54 in which is a gas burner 56 or other convenient heating means.

Moreover chambers 12 and 23 protect both ends of kiln 14 and the upper end of kiln 20 from loss of heat by radiation. It is an important feature according to the present invention that the temperature gradients within the kilns 14 and 20 have no abrupt changes adjacent the ends of the kilns as would inevitably occur if the ends of the kilns were not inclosed by chambers adapted to prevent loss of heat energy by radiation. It is desired also that the lower end of kiln 20 be protected from the introduction of cold air not coming from nozzle 22 and for this purpose, the joint between kiln 20 and the wall of chamber 31 at the point 58 is so constructed as to admit a minimum of air. Chamber 31, also prevents the loss of heat from the lower end of kiln 20 by means of radiation as well as acting as holder for the pot 30.

The joints at the points 60, 62 and 64 between kilns 14 and 20 and the chambers 12 and 23 respectively are also formed to prevent as far as possible the introduction of air into the system except that introduced through the coil 48 and the nozzle 22.

Kilns 14 and 20 may be largely of standard construction and are illustrated as mounted on rotating trunnions 66, 66. The kilns 14 and 20, moreover, may be rotated by any convenient means, worm drives being illustrated for this purpose as indicated at 68, 68. It will be understood that the motors, electric or otherwise, for driving the worm 68 are preferably of variable speed design whereby the speed of kilns 14 and 20 may be readily adjusted or regulated if necessary, to properly co-relate the speed of movement of the solids longitudinally thereof to the speed of movement of the gas current therethrough.

It will be understood that chambers 12, 23 and 31 are formed of materials adapted to prevent loss of heat by conduction through the walls thereof and I have illustrated at 67 a special insulating lining for the chamber 23. Similar linings may be used with the chambers 12 and 13 if desired. Moreover, the kilns 14 and 20 are made of non-heat con-

ducting materials or provided with non-heat conducting or heat insulating layers (not illustrated) to prevent loss of heat through the walls of the kilns and to maintain a uniform 5 temperature gradient within the kilns during operation.

As above described, the lead for making oxides according to the present invention is melted in the pot 10 and preferably by means 10 of waste heat in the outgoing gases. Whenever desirable, however, an auxiliary burner 70 may be installed in chamber 12 beneath the pot 10 to assist in melting or to raise the temperature of the lead in pot 10.

15 Having thus described my invention, I claim:

1. The method of making lead oxide comprising intimately contacting a stream of molten lead in subdivided form with a moving 20 stream of substantially pure air preheated to a temperature of about 800° F.

2. The method of making lead oxide comprising intimately contacting a downwardly flowing stream of molten lead with a counter 25 currently flowing stream of hot substantially pure air, and regulating the rates of flow of said lead and air streams so that a portion of the lead remains unoxidized at the time of its removal from contact with said air stream.

30 3. The method of making lead oxide comprising repeatedly lifting and dropping molten lead transversely of the path of a diagonally upwardly flowing stream of air while moving said lead and oxide diagonally downward countercurrently to the flow of said preheated substantially pure air stream.

4. The method of making red lead comprising moving molten lead with agitation 40 countercurrent to a stream of air, separating lead oxide from said stream and reintroducing said oxide into said stream and forming red lead from said oxide in said stream.

5. The method of making red lead comprising intimately contacting molten lead 45 with a stream of hot air to form lead monoxide, introducing relatively cool air into said stream, and forming red lead from said monoxide in said stream after the introduction of said cooler air.

50 6. The method of making red lead comprising intimately contacting molten lead with a countercurrent stream of air, separating lead oxide from said stream, introducing cooler air into said stream, reintroducing said monoxide into said stream and forming red lead from said monoxide in said stream at a point subsequent to the introduction of said cooler air.

65 7. An apparatus for forming red lead comprising a conduit, means for moving molten lead through a portion of said conduit in a given direction, means for passing a stream of air through said portion of the conduit in a direction opposite to that of said lead, means for agitating said lead in contact with

said air, means for separating lead oxide from said molten lead, means for reintroducing said oxide into said conduit in the second portion thereof, and means for agitating said lead oxide in contact with said stream of air in the second portion of the said conduit.

8. The method of making lead oxide comprising introducing molten lead into the upper end of an inclined rotary kiln, introducing hot air into the lower end of said kiln, lifting and dropping said lead in said current of hot air, and so regulating the travel of the lead and oxide in the kiln with respect to the flow and temperature of said air that a portion of the lead remains unoxidized upon issuing from the lower end of the kiln.

9. The method of making red lead comprising moving melted lead with agitation countercurrent to a stream of hot air, regulating the flow of said lead with respect to the flow and temperature of said air so that a portion of the lead remains unoxidized upon removal from said stream, separating oxide from said unoxidized lead, re-introducing said lead oxide into said stream, and forming red lead from said oxide in said stream.

25 10. The method of making red lead comprising moving molten lead with agitation countercurrent to a stream of hot air, regulating the flow of said lead with respect to said air so that a certain portion of said lead remains unoxidized after its passage through said stream, separating lead monoxide formed in said stream from said unoxidized lead, introducing relatively cooler air into said stream, re-introducing said monoxide into said stream, and forming red lead from said monoxide in said stream at a point intermediate the re-introduction of said monoxide and point of introducing said cooler air.

11. Apparatus for making red lead comprising an inclined rotary kiln, means for introducing hot air into the lower end of said kiln, a second inclined rotary kiln, means for conducting hot gases from the upper end of said first kiln into the lower end of said second kiln, and a lead pot set in the current of hot gases issuing from said second kiln.

12. An apparatus for making lead oxide comprising an inclined rotary kiln, means for introducing hot air into the lower end of said kiln, a lead pot arranged to be heated by the gases after leaving said kiln, a pipe for conducting molten lead connecting said pot with the upper end of said kiln, and means whereby a current of hot gases from said kiln is maintained around said pipe.

13. An apparatus for making lead oxide comprising a pair of inclined rotary kilns set at different levels and inclined oppositely one to the other, means for introducing molten lead through the upper end of the lower of said kilns, means for introducing hot air into the lower end of the lower of said kilns, means at the lower end of said lower kiln for

70

75

80

85

90

95

100

105

110

115

120

125

130

separating metallic lead from lead oxide, means for introducing said oxide into the upper end of said upper kiln, and chambers surrounding the ends of said kilns, one of said chambers serving to conduct gases from the lower to the upper of said kilns and all of said chambers acting to prevent radiation from the ends of said kilns.

14. An apparatus for forming lead oxide comprising a rotary kiln inclined to the horizontal sealed against the leakage of air thereto, an air preheater, a pipe for introducing hot air from said preheater into the lower end of said kiln, a melting pot and connections for introducing molten lead into the upper end of said kiln, pockets on the interior of said kiln arranged for lifting and dropping said molten lead in its passage through said kiln, and a valved pipe for introducing cooler air into said kiln intermediate the points of introducing said hot air and said lead.

15. The method of making lead oxide comprising intimately contacting countercurrently flowing streams of molten lead and preheated substantially pure air in a kiln, the temperature of which is maintained at about 700° F.

16. The method of forming red lead comprising intimately contacting countercurrently flowing streams of molten lead and a preheated oxidizing gas stream at an elevated temperature to produce lead monoxide, and intimately contacting lead monoxide thus formed with said preheated oxidizing gas stream at a still higher temperature to produce red lead.

17. The method of forming red lead comprising maintaining a temperature of about 700° F. in a kiln while intimately contacting countercurrently flowing streams of molten lead and preheated air therein, and maintaining a temperature of about 840° F. in a second kiln while intimately contacting lead monoxide formed in said first kiln with said countercurrently flowing stream of preheated oxidizing gas.

18. The method of converting lead into red lead comprising intimately contacting molten lead with a flowing stream of substantially pure air preheated to a temperature of about 800° F., in a kiln maintained at a temperature of about 700° F., and converting the lead monoxide thus formed into red lead by intimately contacting it with a stream of preheated air in a second kiln maintained at a temperature of about 840° F.

19. The method of making red lead comprising intimately contacting a downwardly flowing stream of molten lead with a countercurrent upwardly flowing stream of preheated air in a closed kiln, so regulating the rates of travel of lead and air through the kiln that a mixture of unoxidized lead and lead monoxide is removed from the lower end of the kiln,

separating the lead from the lead monoxide, and passing the lead monoxide downwardly through another closed kiln in intimate heat-transferring contact with a countercurrently flowing stream of hot air.

20. The method of making red lead comprising passing molten lead downwardly through a kiln in direct heat-transferring contact with a countercurrently flowing stream of preheated air, passing lead monoxide formed in said kiln countercurrently through another kiln in direct heat-transferring contact with said air stream, and utilizing the waste heat in said air stream to reduce said lead to a molten state prior to introducing it into said first named kiln.

In testimony whereof, I affix my signature.

CARL J. WRIGHT.

70

85

90

95

100

105

110

115

120

125

130